

# UNITED STATES PATENT OFFICE.

HELMUT KLEVER, LUDWIG CARL LAUTENSCHLÄGER, AND OSWALD HELMUTH GÖHRING, OF KARLSRUHE, GERMANY, ASSIGNEES, BY MESNE ASSIGNMENTS, TO THE CHEMICAL FOUNDATION, INC., A CORPORATION OF DELAWARE.

## PROCESS OF MANUFACTURING LUBRICATING-OILS.

1,350,814.

Specification of Letters Patent. Patented Aug. 24, 1920.

No Drawing.

Application filed February 14, 1916. Serial No. 78,311.

To all whom it may concern:

Be it known that we, HELMUT KLEVER, LUDWIG CARL LAUTENSCHLÄGER, and OSWALD HELMUTH GÖHRING, Ph. D., chemists, citizens

5 of the German Empire, residing at Karlsruhe, in the Grand Duchy of Baden, Germany, have invented certain new and useful Improvements in Processes of Manufacturing Lubricating-Oils, of which the following is a specification.

10 It is well known that coal tar oils yield lubricating agents of inferior quality. In accordance with our invention however the viscosity of coal tar oils is increased and it is possible to compensate the lack in adhesive qualities by the effects of an increase in toughness. In accordance with our invention we have discovered that the viscosity of coal tar oils may be increased by the

15 condensation and polymerization of compounds contained therein and capable of such reaction. These points are produced by heating the oils for some time at high temperatures. The oils are thus converted

20 into valuable pressure lubricating oils. This is due to the fact that coal tar oils, particularly the anthracene oils and the naphthalene oils, and the distillation products of coal tar pitch, containing bases and phenols

25 of high molecular weight are capable of condensation by prolonged heating. Some of the bases liberate ammonia, while the phenols liberate water. This heating of the coal tar oils is preferably effected under

30 pressure or by allowing the condensed vapors to flow back, so as to avoid losses. The oils obtained are the more viscous or less liquid, the longer they have been heated and the higher the temperature employed. By

35 increasing the amount of air admitted during the heating process, the oils will be converted into pitch. Air should therefore be excluded as much as possible from the reactions going on during the heating process.

40 The admission of a very limited amount of air, which is governed by the origin and the composition of the oils employed and which has to be ascertained by a preliminary test, promotes the reactions mentioned.

45 The admission of air must be adjusted in such a manner that it does not convert the oils into pitch even to an inconsiderable extent.

50 For the purpose of producing oils of lighter colors it is of advantage to operate

in an atmosphere of indifferent gases, for instance hydrogen, nitrogen, carbon dioxide or the like. The yield is substantially quantitative.

55 If the fractions of lower boiling point are distilled off from naphthalene oils until a residue having a flash point of about 130 degrees C. remains in the retort, this residue is a thin liquid and of inferior quality as a lubricant. If however, the naphthalene oils are submitted to the heating process in accordance with my invention and particularly under pressure and if the easily inflammable components are then distilled off at their respective boiling points, a residue 70 is obtained which constitutes a lubricating oil of high viscosity. In this manner even the lighter distillation products of coal tar are suitable for treatment by this process.

60 Inasmuch as the thickening of the oil is 75 chiefly due to the condensation of bases and of phenols, it is obvious that coal tar oils can be particularly adapted for the process of our invention by increasing the amount of bases and phenols therein according to 80 well known processes or by adding such components including those which may be obtained from tar oils of other origin, as for instance from wood tar. As a matter of fact the coal tar oils which have been enriched in bases and phenols in accordance with well known processes, show the thickening effect of the process of our invention in a particularly marked manner.

65 The bases and phenols mentioned may 85 also be heated by themselves in accordance with the present process, masses similar to petroleum pitch being obtained thereby which may be added to the coal tar oils in order to produce lubricants of high viscosity. In a general way the productivity of our process may be improved by inspissating part of the coal tar oils to be treated, to a very high degree by itself. A product of the desired average viscosity may be obtained by the addition of the inspissated product to oils not so treated.

70 The processes of condensation and polymerization described may be assisted by the addition of small amounts of catalysts, for 105 instance one to two per cent. thereof. Of such catalysts we may mention, Florida earth, kieselguhr, animal charcoal, powdered graphite, chlorides of metals, such as the chlorides of aluminium, zinc, iron, cadmium, cop- 110

per proto-chlorid and the like, also metallic powder, powdered metal oxids and metal hydroxids, such as those of iron, nickel, cobalt, chromium, aluminium, zinc, copper, 5 lead and the like, or the oxids and hydroxids of the alkali and alkaline earth metals.

By the treatment in accordance with our process the congealing point of the final products is improved as a general rule as 10

compared with those of the crude material. The crystalline bodies, such as anthracene, indene, picene and the like which separate out when the coal tar oils are cooled and cause so much trouble, are considerably less 15 noticeable in the oils treated according to our invention. In accordance with the origin and the composition of the coal tar oils employed the heating may be carried out in such a manner as to avoid such separations 20 entirely, the oils solidifying homogeneously.

When it is desired to produce oils of very low congealing point it is preferable to remove the products which crystallize most easily, from the crude oils in accordance 25 with known processes, by distillation for instance of the fractions containing the precipitating bodies or by keeping them for a long time at a low temperature, and then submitting the oils to suction or to centrifugal 30 action. These operations are likewise applicable to the inspissated oils.

The oils obtained according to our process are especially characterized by their very faint odor as compared with the original 35 oils. They are eminently adapted for all lubricating purposes particularly for lubrication under pressure.

#### Examples.

40 I. 200 pounds anthracene oil II (fat oil) viscosity about 19 degrees Engler (+20 degrees C.) and with a solidifying point of -7 degrees C. are heated for 24 hours in a pressure boiler at about 350 degrees C.; 45 after cooling a difficultly flowing lubricating oil is obtained of a viscosity of about 55 degrees E. (+20 degrees C.) and about 4.5 to 4.7 viscosity Engler (+50 degrees C.), the solidifying point being unchanged while the 50 yield is substantially quantitative. During solidification considerably less crystalline separations are noticed than in the crude oil.

II. Heat 200 pounds anthracene oil II (fat oil) of a viscosity of about 19 degrees 55 Engler (+20 degrees C.) in a pressure boiler for about 24 hours at about 380 degrees C. A high viscid oil is obtained, possessing the viscosity of about 10 to 15 degrees E., at +50 degrees C.

60 By dissolving 132 pounds of this highly viscid oil in 68 pounds of the untreated crude oil, an oil having the viscosity of about 55 to 60 degr. E. (+20 degrees C.) is obtained.

65 III. Heat 200 pounds of fat oil of a vis-

cosity of about 19 degrees Engler (20 degrees C.) under pressure at about 420 degrees C. from 7 to 10 hours. A resin-like tough mass is obtained which is dissolved in an equal amount of anthracene oil I from 70 which the naphthalene fractions have been removed resulting in an oil of the viscosity 90 to 100 degrees Engler (20 degrees C.).

IV. 196 to 198 pounds of the naphthalene fraction of the tar boiling point 200 to 280 75 degr. C. (measured in the vapors) and of a viscosity of about 1.5 degr. Engler, are heated for 24 hours at 350 degrees C. in a pressure boiler with 2 to 4 pounds of iron powder or oxid of iron powder. After cooling the product is distilled until the boiling point 280 degrees C. (determined in the vapors) has been reached. There remain about 50 to 56 pounds of an oil possessing the viscosity of about 40 degrees Engler (20 80 degr. C.).

By distilling off 72 per cent. of the fractions of lower boiling point from the untreated original oil, a residue of about 5 to 7 degr. Engler (20 degrees C.) was obtained. 90

V. 196 to 198 pounds of dehydrated anthracene oil II (fat oil) of viscosity about 19 degrees E. (20 degrees C.) are heated for 24 hours with the exclusion of air under a reflux condenser with 2 to 4 pounds of 95 powdered iron or oxid of iron. The boiling point of the liquid is about 315° C. at the beginning of the boiling and rises during the boiling to about 325 degrees C. An oil in substantially quantitative proportions is 100 produced possessing the viscosity of about 40 to 50 degrees E. at +20 degrees C. By allowing the boiling to continue for 48 hours, an oil results having at +20° C., a viscosity of about 50 to 60 degrees Engler 105 and at +50° C. the viscosity of 4.5 to 5.0 degr. E. The oil produced under these conditions is lighter colored than the oils obtained in accordance with the preceding examples. It is clearly soluble in benzol and 110 xylol and with faint fluorescence in mineral oils.

VI. 196 to 198 pounds dehydrated anthracene oil II (fat oil) of a viscosity of about 19 degrees Engler (+20° C.) are boiled under a reflux condenser for 24 hours with 115 from 2 to 4 pounds of iron powder or powdered oxid of iron. According to the nature of the oil employed air is admitted to the boiling oil during a certain time which 120 has been ascertained by a previous test. The lower the boiling point of the liquid the longer the air may be allowed to remain in contact with the oil as a general rule, without the formation of pitch-like by-products which are insoluble in benzol. The viscosity of the final product treated with air, is considerably higher than that of an oil boiled with the exclusion of air. By 125 using the anthracene oil mentioned and com- 130

mencing to boil at about 315° C. (measured in the liquid) a viscosity of about 40 to 45 degrees Engler (+20° C.) was produced after 24 hours with the exclusion of air, while 5 on the admission of a moderate amount of air which was obtained by a liquid seal merely for equalizing the difference of air pressure within and without the boiler, a viscosity of about 50 to 55 degrees Engler (+20 degr. C.) was produced.

VII. 186 pounds of anthracene oil II (fat oil) of a viscosity of about 19 degr. E. (+20° C.) are boiled with 10 pounds phenol from wood tar from which the fractions 10 boiling up to about 280 degrees C. had been removed, and with 4 pounds of iron powder with the exclusion of air under a reflux condenser for 24 hours, resulting in a lubricating oil which possesses the viscosity of 15 about 50 to 60 degrees Engler (+20° C.)

VIII. About 42 pounds of bases and 24 pounds of phenol obtained from anthracene oil II (fat oil) by means of alkalis or by the enriching of certain fractions, are mixed and 20 are heated with the exclusion of air for 24 to 48 hours with about 4 pounds of iron powder or iron oxid powder at 320 to 350 degrees C. under reflux or under pressure. The condensing reaction takes place with the 25 liberation of ammonia and of water. A tough, brownish black mass is obtained which is soluble in tar oils with a great increase of viscosity. Ten per cent. of the product heated for 24 hours at 350° C. under 30 pressure is soluble in fat oil of a viscosity of about 19 degrees Engler (+ 20° C.) and produces a lubricating oil having a viscosity of about 45 degrees Eng. (+ 20° C.)

We claim:—

1. The process of manufacturing lubricating oils from coal tar oils or distillates of coal tar pitch embodying chiefly bases and phenols, consisting in condensing and polymerizing the components of such substances 40 by heat under pressure, and avoiding losses by evaporation during the heating of the substances.

2. The process of producing lubricants from coal tar oils or distillates of coal tar 45 pitch, which consists in heating such product under reflux and preventing loss by evaporation during the heating of the product.

3. The process of producing lubricants from coal tar oils or distillates of coal tar 50 pitch which consists in heating such product under reflux in the presence of a catalyst and preventing loss by evaporation during the heating of the product.

4. The process of producing lubricants 55 from coal tar or distillates of coal tar pitch which consists in heating such product under reflux in the presence of iron oxid and preventing loss by evaporation during the heating of the product.

5. The process of producing lubricants 65 from coal tar or distillates of coal tar pitch which consists in heating such product under reflux in the presence of powdered oxid of iron and preventing loss by evaporation during the heating of the product.

6. The process of producing lubricants 70 from coal tar oils or distillates from coal tar pitch embodying chiefly bases and phenols, consisting in heating the components of the substance in an atmosphere of indifferent gases under pressure, and preventing loss by evaporation during the heating of the substance.

7. The process of producing lubricants 75 from coal tar oil or distillates from coal tar pitch embodying chiefly bases and phenols consisting in heating the constituents of the material in an atmosphere of indifferent gases under pressure in the presence of a catalyst and preventing loss by evaporation 80 during the heating operation.

8. The process of producing lubricants 85 from coal tar oil or distillates from coal tar pitch embodying chiefly bases and phenols consisting in heating the constituents of the material in an atmosphere of indifferent gases under pressure in the presence of iron oxid and preventing loss by evaporation during the heating operation.

9. The process of producing lubricants 90 from coal tar oil or distillates from coal tar pitch embodying chiefly bases and phenols consisting in heating the constituents of the material in an atmosphere of indifferent gases under pressure in the presence of powdered oxid of iron and preventing loss by 95 evaporation during the heating operation.

10. As a new article of manufacture, a lubricating oil consisting of condensed and polymerized coal tar oils or distillates from 100 coal tar pitch having high viscosity and being soluble in tar oils, benzol, xylol, and mineral oils.

11. As a new article of manufacture, a lubricant consisting of condensed and polymerized bases and phenols and coal tar oils 110 or distillates from coal tar pitch having high viscosity and being soluble in tar oils, benzol, xylol, and mineral oils.

In testimony whereof we have hereunto 115 set our hands in presence of two subscribing witnesses.

HELMUT KLEVER.

LUDWIG CARL LAUTENSCHLÄGER.

OSWALD HELMUTH GÖHRING.

Witnesses for Helmut Klever and Ludwig Carl Lautenschläger:

RICH. WEINGAND,  
C. INNESS BROWN.

Witnesses for Göhring:

HENZE D. DAMM,  
HENRY QUAD FLÜG.